

April 27, 1943.

P. GÖRLICH

2,317,754

METHOD OF PRODUCING SECONDARY ELECTRON EMITTING CATHODES

Filed July 31, 1941

Fig. 1



Fig. 2



INVENTOR  
BY Paul Görlich  
Singer, Ehler, Stern & Berling  
ATTORNEYS

## UNITED STATES PATENT OFFICE

2,317,754

## METHOD OF PRODUCING SECONDARY ELECTRON EMITTING CATHODES

Paul Görlich, Dresden, Germany; vested in the Alien Property Custodian

Application July 31, 1941, Serial No. 404,811  
In Germany July 31, 1940

6 Claims. (Cl. 250—27.5)

The invention relates to improvements in a method of producing secondary electron emitting cathodes.

It is known that metals whose surface is covered with layers of earth alkali metals belonging to the second group of the periodic system, or with layers of earth metals belonging to the third group of the periodic system, have the property of emitting a high amount of secondary electrons. The amount of the secondary electron emission depends upon the thickness of the metal layer which has been deposited upon the surface of the metal. The control of the thickness of the layer during the production of secondary electron emitting cathodes is therefore of extremely great importance, particularly in the case of secondary electron multipliers, in which a number of secondary electron emitting electrodes are arranged one after another.

It is an object of the invention to produce secondary electron emitting cathodes and particularly to provide the same with an exterior metal layer of a thickness producing the best results.

Another object of the invention is to apply the metallic layer to the electrode body in a special apparatus and prior to the assemblage of the various cathodes in the tube in such a manner, that during the period the metal is precipitated by vaporisation or during two successive periods of precipitation respectively, the layers under construction are being bombarded with primary electrons for testing the sensitiveness of the layers. The precipitation by evaporation is interrupted when the maximum sensitiveness has been reached. In this manner, the surface of each electrode may be provided separately with a metallic layer, but it is also possible to give the apparatus such a construction that at the same time a plurality of electrodes are provided on their surface with the respective metal layer.

When the secondary electron emitting layers are produced in the manner just described it is hardly avoidable that the secondary electron emitting electrodes during their assemblage in the multiplier tube come in touch with the air, particularly with the oxygen contained in the same. The possible oxidation of the surface layer is a disadvantage insofar as it influences the energy necessary to produce the electron emission, which energy has to be increased considerably when the metallic layer on the electrode becomes oxidized. It is therefore another object of the present invention to counteract or compensate any oxidation of the metallic surface

layer on the electrodes. After the various electrodes have been installed in the multiplier tube, they are subjected to a glow discharge, preferably in the presence of a rare gas or another chemically inactive gas. Such a glow discharge between the electrodes reduces any oxide which might have been formed and thus any loss in sensitiveness will have been regained. The glow discharge has the additional advantage that it liberates any adsorbed or absorbed gases and thereby makes the electrodes independent of the uncontrollable action of such gases.

Preferably, the glow discharge is maintained a sufficient length of time until the oxide layer formed during the period the electrodes were subjected to the influence of the air is entirely reduced. The necessary operating conditions under which the glow discharge is practiced, particularly the required length of time, can easily be determined by tests. However, it is also possible to measure in predetermined periods of time the sensitiveness by means of primary electrons as mentioned previously.

The method according to the invention is employed with a device shown in the drawing. The drawing however only shows an example of the device according to the invention.

Figure 1 illustrates the manufacture of the surface metal layer of the secondary electron emitting electrodes. In bulb 1 the secondary electron emitting electrodes 3, 4, 5, 6 are attached to a support 2. The metal which is to be precipitated by vaporization, for instance an alkali metal, is fixed to the heated filament 7. After a certain time of vaporization the vaporization will be stopped in order to measure the secondary electron current. To this effect there is a potential of 120 volts on the one side between the heated filament 7 and the secondary electron emitting electrodes and a potential of 80 volts on the other side between the secondary emitting electrodes 3, 4, 5, 6 and the end of the auxiliary electrode 8.

As soon as the secondary electron emitting electrodes 3, 4, 5, 6 have reached the maximum sensitiveness they will be assembled in the multiplier tube 9 as shown in Figure 2. The assemblage of secondary electron layers in a multiplier tube is not limited to the example shown in Figure 2. In the multiplier tube 9 part 10 represents the light sensitive cathode which is illuminated by the light falling in in the direction of the arrows. No. 11 shows an anode in form of a grid, having also the faculties of emitting secondary electrons. After having passed the grid 11 these electrons

strike (one after the other) the secondary electron emitting layers 3, 4, 5, 6 (—) causing on their way the emission of more and more secondary electrons and finally strike the electrode 12 and at last give away their energy to anode 13.

In the above described example the manufacturing method according to the invention was shown having 4 secondary electron emitting electrodes. In the same way it will be possible to manufacture less or more than 4 secondary electron emitting electrodes.

What I claim is:

1. A method for producing secondary electron emitting electrodes comprising precipitating a thin surface layer of an alkali metal on a metal base prior to the installation of the electrodes in an electron multiplier, installing the electrodes having said thin layer thereon in said electron multiplier, and then subjecting the electrodes to a glow discharge until any oxidation of said thin layer has been reduced.

2. A method for producing secondary electron emitting electrodes comprising precipitating a thin surface layer of an alkali metal on a metal base prior to the installation of the electrodes in an electron multiplier, continuously controlling the thickness of the precipitated layer by measuring the sensitiveness of the secondary electron emission until the maximum sensitiveness is obtained, installing the electrodes having said thin layer thereon in said electron multiplier, and then subjecting the electrodes to a glow discharge until any oxidation of said thin layer has been reduced.

3. A method for producing secondary electron emitting electrodes comprising precipitating a thin surface layer of an alkali metal on a metal base prior to the installation of the electrodes in an electron multiplier, intermittently controlling the thickness of the precipitated layer by meas-

uring the sensitiveness of the secondary electron emission until the maximum sensitiveness is obtained, installing the electrodes having said thin layer thereon in said electron multiplier, and then subjecting the electrodes to a glow discharge until any oxidation of said thin layer has been reduced.

4. A method for producing secondary electron emitting electrodes comprising precipitating a thin surface layer of an alkali metal on a metal base prior to the installation of the electrodes in an electron multiplier, installing the electrodes having said thin layer thereon in said electron multiplier, and then subjecting the electrodes to a glow discharge in the presence of a rare gas until any oxidation of said thin layer has been reduced.

5. A method for producing secondary electron emitting electrodes comprising precipitating a thin surface layer of an alkali metal on a metal base prior to the installation of the electrodes in an electron multiplier, installing the electrodes having said thin layer thereon in said electron multiplier, and then subjecting the electrodes to a glow discharge in the presence of a chemically inactive gas until any oxidation of said thin layer has been reduced.

6. A method for producing secondary electron emitting electrodes comprising precipitating a thin surface layer of an alkali metal on a metal base prior to the installation of the electrodes in an electron multiplier, installing the electrodes having said thin layer thereon in said electron multiplier, then subjecting the electrodes to a glow discharge until any oxidation of said thin layer has been reduced, and controlling the effect of the glow discharge by measuring intermittently the sensitiveness of the secondary electron emission.

PAUL GÖRLICH.